

## UNITED STATES PATENT OFFICE

CHARLES W. ANDREWS, OF CHICAGO, ILLINOIS, ASSIGNOR TO H. A. BRASSET & COMPANY, OF CHICAGO, ILLINOIS, A CORPORATION OF ILLINOIS

## METHOD FOR MAKING COKE

No Drawing.

Application filed September 22, 1928. Serial No. 307,786.

This case relates to a new and improved method for making coke and more particularly to a composition or mixture for use in making coke.

It is well known in the art that good coke, especially that suitable for metallurgical purposes is usually made by the addition of low volatile coals to the usual high volatile coal before the coking operation. Such low volatile coal usually runs from ten to twenty percent of the total mass and serves to make the coke more blocky and better adapted for usual requirements. It is also known that the grinding and mixing together of the high and low volatile coals before the coking operation has very considerably improved the structure of the coke as compared with that made without the grinding and mixing. In such usual methods, however, it has been found that the finest part of the coal dust is not desirable for coke making and hinders rather than helps in the production of satisfactory coke.

Large quantities of anthracite culm are available and also of coke breeze. These are both practically waste materials and any method of making coke which will utilize them will result in considerable savings in the cost of the coke.

It is an object of the present invention to provide a new and improved method and mixture of materials for the production of coke.

It is a further object to provide a sizing and proportioning of materials adapted for use in making coke.

It is also an object to provide a method and mixture adapted to utilize anthracite culm or coke breeze in the production of coke.

Other and further objects will appear as the description proceeds.

I have found by experiment that if the fineness of the anthracite culm or dust and of coke breeze is held within certain limits and the percentage added to the high volatile coal is also held within certain limits I accomplish the manufacture of a coke which is equal to or better than that obtained from usual mixtures of high and

low volatile coal under the normal operations of a coke plant.

My experiments show that a percentage varying from about 5 to 15 of the total mass constitutes the most desirable operating limits for the use of anthracite culm or coke breeze. This material also should be crushed so as to fall between the limits of approximately one hundred percent passing through an eighth inch mesh to approximately one hundred percent passing a standard forty mesh sieve. By the statement approximately one hundred percent I intend to cover a variation of a few percent which will not seriously affect the operation and quality of the coke.

The remaining 85 to 95 percent consists of high volatile coal and may be crushed to the ordinary fineness used in present coke oven practice, namely, about eighty percent or more through a one eighth inch screen and approximately ninety five percent through a quarter inch screen. I have found, however, that if practically all of the high volatile coal is sized to pass through a one eighth inch screen the quality of the coke is materially benefited. This fine grinding of the high volatile constituent is contrary to the usually accepted practice as has been stated above, but has been found to give a better coke where the low volatile constituent of the coke comprises anthracite culm or coke breeze of the sizes and proportions I have given above.

Where reference is made to material of any specific fineness, as eighty percent or more through a one-eighth inch mesh screen, it is meant that the material is varied in size as the result of a usual crushing or grinding operation with the maximum sizes such as to conform to the stated screen test.

My experience indicates that the finest grade of coke is made where the high volatile constituent practically all passes through an eighth inch mesh and constitutes substantially 87½ to 90 percent of the whole and the anthracite dust or culm or the coke breeze is crushed to forty mesh size and constitutes from 10 to 12½ percent of the total used.

My experiments have demonstrated that

the porosity of the coke produced by this method may be selectively varied over a comparatively wide range, or from approximately 50 percent to 58 percent. This variation is 5 accomplished by varying the size of the anthracite or coke dust, the forty mesh crushing giving the lowest porosity. This is a matter of great importance as it is recognized in blast furnace practice that the porosity of 10 the coke should be varied depending upon the nature of the iron desired, for example, foundry iron or basic iron.

The coke made when the anthracite or coke breeze is only crushed to pass a one sixteenth 15 inch mesh is not quite so good but is, nevertheless, up to the standard of coke made by usual methods.

The coke made according to my invention is not only of good structure as demonstrated 20 by the fact that a larger percentage remains on an inch screen after the usual tumbler test than remains of coke made by normal methods, but the coke itself also shows better cell structure.

25 An important feature is the use of low volatile carbonaceous material such as anthracite culm or coke breeze which are practically waste materials which thereby reduce the cost of the coke.

30 While I have described in detail certain preferred sizes and proportions of material by way of example, it is to be understood that I contemplate such changes and modifications as come within the spirit and scope of 35 the appended claims.

I claim:

1. The method of making coke which comprises mixing a mixture comprising up to fifteen percent of low volatile solid combustible carbonaceous material sized to substantially all pass a sixteenth inch mesh screen and high volatile coal crushed to a size such that at least approximately ninety percent will pass a quarter inch mesh screen, and subjecting the mixture to a coking operation. 45

2. The method of making coke which comprises mixing approximately ten percent of low volatile solid combustible carbonaceous material sized to approximately all pass a forty mesh screen and approximately ninety percent of high volatile coal crushed to approximately all pass through an eighth inch mesh screen, and subjecting the mixture to a coking operation. 50

55 3. A coking mixture comprising seven and a half to fifteen percent of low volatile solid combustible carbonaceous material sized to substantially all pass a sixteenth inch mesh and eighty-five to ninety-two and a half percent of high volatile coal crushed to a size such that at least approximately eighty percent will pass an eighth inch mesh screen and approximately ninety-five percent will pass a quarter inch mesh screen. 60

65 4. A coking mixture comprising approxi-

mately ten percent of coke breeze crushed to practically all pass a forty mesh screen and approximately ninety percent of high volatile coal crushed to a size to practically all pass an eighth inch mesh screen. 70

5. The method of making coke of selected porosity which comprises mixing high volatile coal crushed to a size such that approximately ninety percent will pass a quarter inch mesh screen, together with low volatile solid combustible carbonaceous material making up from five to fifteen percent of the entire mixture, said low volatile material being crushed to approximately all pass a sixteenth inch mesh screen, and selectively crushing 75 said low volatile material, before said mixing, between said sixteenth inch size as an upper limit, and a lower limit of a size such that substantially all will pass a forty mesh screen, depending upon whether a more or less porous product is desired, the coarser sizes giving more porosity and, the finer sizes giving less porosity, and subjecting the mixture to a coking operation. 80

Signed at Chicago, Illinois, this 19th day 85 of September, 1928.

CHARLES W. ANDREWS.

95

100

105

110

115

120

125

130